

## UNITED STATES PATENT OFFICE.

ANDRÉ GEYER, OF PARIS, FRANCE.

## ALUMINUM ALLOY.

No Drawing.

Application filed September 11, 1922. Serial No. 587,582.

To all whom it may concern:

Be it known that I, ANDRÉ GEYER, engineer, citizen of the Republic of France, residing in Paris, France (and whose post-office address is 14 Rue Civiale), have invented certain new and useful Improvements in Aluminum Alloys; and I do hereby declare the following to be a full, clear, and exact description of the invention, such as 10 will enable others skilled in the art to which it appertains to make and use the same.

This invention relates to aluminum alloys and processes for the manufacture thereof, and has for its object the manufacture of a 15 light alloy, the basis of which is aluminum, which possesses superior qualities of resistance to rupture, of elasticity and of extensibility, together with practically negligible coefficients of dilation and contraction, and 20 a low density. This alloy which consists essentially of the combination of the following constituents: aluminum, copper, manganese, magnesium, lead and carbon, is free from the striæ or filaments of oxide of 25 aluminum that form lines of rupture and lends itself very well to machining and to autogenous welding; it is unoxidable and susceptible of acquiring a beautiful polish.

According to this invention the process of 30 manufacturing this alloy consists essentially in combining carbon with the metallic constituents of the alloy in the bath, while preventing the oxidation of the metal by shielding the surface of the bath from the effects 35 of the contact of the air. The combination of the carbon in graphitic form is advantageously obtained by incorporating with the bath finely powdered carbon, derived, for example, from charcoal and assisted by 40 stirring; the surface of the bath being shielded from the action of air during this carbon treatment by means of a protecting layer, for example of charcoal floating on the surface of the bath, or by any other suitable or known method.

In practice, the operation is performed as follows:

The cupro-manganese mixture is first prepared with the required proportion, the 50 greatest portion of the aluminum intended to constitute the alloy is then melted, and powdered and broken charcoal is introduced in the aluminum bath from the beginning of the melting. The previously prepared 55 cupro-manganese mixture is then added to the bath, and the temperature is raised. The

remainder of the aluminum is subsequently added and the temperature is then allowed to fall somewhat. Finally the magnesium and the lead are added and the metallic alloy 60 so obtained is cast into moulds.

The operation is advantageously effectuated in a covered crucible or the like, which is only uncovered during the time necessary for the successive additions of the materials 65 and for the mixing. The latter must be frequent, and care must be taken to add to the bath new quantities of powdered charcoal at each opening of the crucible or the like, so as to ensure the proper combination of the 70 carbon with the alloy. As it has been stated above, all oxidation of the metal of the bath will be prevented by the layer of broken-up charcoal floating on its surface.

Finally, the metal is suitably reheated 75 before use.

The following typical composition of a 80 rupture resisting alloy is given as a particular example of an alloy according to this invention:

|           |        |
|-----------|--------|
| Aluminum  | 93.92  |
| Copper    | 4.25   |
| Magnesium | 0.79   |
| Manganese | 0.80   |
| Lead      | 0.24   |
| Carbon    | 85     |
|           | 100.00 |

The alloy comprises also traces of silicon and, it may be, of iron, which may be contained as impurities in the metals used 90 constituents.

Once reheated and rolled, for instance in the shape of plates of 20 mm. in thickness, the metal obtained gives approximately the 95 following characteristic coefficients:

|                             | kg.  |
|-----------------------------|------|
| Resistance to rupture       | 43.5 |
| Coefficient of elasticity   | 25   |
| Coefficient of extension    | 20.3 |
| Coefficient of constriction | 0.38 |
| Density (about)             | 2.78 |

It will be understood that by suitable reheating and rolling, the above mentioned coefficients may be somewhat varied.

The particular process of manufacture of this alloy will now be described, as an example:

The cupro-manganese mixture is prepared in the proportions of 4.25 of copper to 0.80 110 of manganese. About three-quarters of the whole aluminum are melted, powdered and

broken coal being introduced into the mass, and the said previously prepared cupro-manganese mixture is added. The temperature of the bath is raised to about 950° C. 5 for nearly two hours. The remaining aluminum is then added and the temperature is allowed to fall to about 800° C. The mixture is well stirred and the heating continued at the same temperature. Finally 10 the lead and the magnesium are added, taking care that the magnesium does not rise to the surface of the bath. The metal is stirred and skimmed and the alloy obtained is cast into ingots or pigs, with the usual 15 precautions for casting aluminum. The metal is finally reheated during about 2 to 3 hours.

The alloy so manufactured lends itself to direct machining by rolling, drawing, etc.,

the metal having obtained its characteristic properties without quenching or other particular heat treatment:

I claim:

1. A process of manufacturing an aluminum alloy containing copper, manganese, magnesium and lead which comprises maintaining the mixture molten while protected on its surface by a layer of finely divided carbon containing material and stirring the metal while so protected to cause the carbon to enter the metal.

2. A strong, ductile alloy of light weight composed of about 93.92% aluminum, 4.25% copper 0.79% magnesium, 0.80% manganese and 0.24% lead and carbon.

In testimony that I claim the foregoing as my invention, I have signed my name.

ANDRE GEYER.

35